

## UNITED STATES PATENT OFFICE

1,923,502

PROCESS AND PRODUCT FOR PROTECTING  
ALUMINIUM, MAGNESIUM, ZINC AND  
THEIR ALLOYS AGAINST CORROSION

Pierre Prier, Clichy, France

No Drawing. Application April 6, 1931, Serial No.  
528,250, and in France April 24, 1930

## 6 Claims. (Cl. 148—6)

This invention has for object improvements in the process and product forming the subject-matter of the United States Patent application No. 401,384. In this patent application have been set forth the conditions which are necessary and sufficient for causing a deposit to be made on the metals it is desired to protect.

The metals used for this protection are given by way of indication, viz: vanadium, molybdenum, tungsten, titanium, uranium, niobium, manganese and also chromium which as all the preceding metals possesses the required qualities and has in particular, the property of forming chromic salts and chromates.

Generally speaking, for protecting articles against corrosion, use was made of the action of an alkaline bath containing one of the alkaline salts of the most oxygenated oxide of a metal capable of forming at least two oxides, the most oxygenated being soluble in alkaline solutions and the less oxygenated not being soluble therein.

The present invention has particularly for object a process derived from the preceding one and having special advantages in that it is of great efficiency and can be commercially carried out.

It has also for object a product serving to prepare the bath to be used for obtaining the required protecting deposit.

This product comprises in a mixture with the fixing product the main ingredient of which is vanadium, molybdenum, etc., an oxy-acid salt or an organic oxy-compound and an alkali phosphate and, preferably, a certain quantity of alkali carbonate, or of an alkali, or of another basic salt, such for instance as cyanides of sodium or potassium.

By dissolving this product in water, a bath is obtained which, when brought to boiling point, will serve to treat articles made of aluminium, magnesium or zinc, or their alloys, on which a protecting deposit is to be formed.

It has been found that articles made of aluminium or aluminium alloy which are to be protected give rise in the active bath according to the above mentioned patent application to a flaky or flocculent deposit of alumina soluble in the hot state in the form of aluminate, which is decomposed by cooling.

The formation of aluminium hydroxide hinders fixation by partially concealing the metal, this increasing the duration of the operation and giving a deposit which is insufficiently homogeneous.

It has been found that for eliminating this alumina, the presence of oxy-acid salts or of or-

ganic oxy-compounds such as malic acid, tartaric acid, citric acid, sugar, starch, etc., or of an alkali phosphate, alone or to which is added a basic body such as alkali carbonate or alkali, is necessary.

It prevents the formation of alkaline aluminate either by reducing aluminium to the condition of soluble negative complexions in the case of oxy-compounds, or by causing precipitation of a dense alumina phosphate insoluble in the hot state in the case of alkali phosphates.

Consequently, the time necessary for the formation of the protecting layer is diminished, and the homogeneity of the latter, and therefore its resistance, are increased.

The bath can serve indefinitely by enriching it with a mixture composed of an active salt, an oxy-compound, an alkali phosphate and an alkali carbonate or an alkali.

The alkali content must remain proportional to the fixing salt content.

By way of example, the following proportion is suitable:

|                                       | Per cent | 80 |
|---------------------------------------|----------|----|
| Phospho-chromate and sulpho-molybdate | 1.50     |    |
| Tri-phosphate of sodium               | 0.40     |    |
| Carbonate of sodium                   | 1.80     |    |
| Tartrate of sodium                    | 1.80     |    |

The preceding example is given by way of indication and not in a limiting sense.

For producing on zinc and its alloys a protecting deposit according to the invention, the alkaline and fixing salts indicated above must be used in a similar proportion.

By way of example, the following composition allows to obtain a satisfactory protecting deposit on zinc or zinc alloys:

|                                       | Per cent | 95 |
|---------------------------------------|----------|----|
| Phospho-chromate and sulpho-molybdate | 1.50     |    |
| Tri-phosphate of sodium               | 0.50     |    |
| Carbonate of sodium                   | 1.20     |    |
| Tartrate of sodium                    | 1.50     |    |

The above example is given by way of indication and is not to be considered as limitative.

The protecting layer formed constitutes an excellent fixing base for any varnish and paint.

What is claimed:

1. A process for protecting aluminium, magnesium, zinc and their alloys against corrosion, which consists in forming a protecting layer on articles made of these metals or alloys by the action of a hot bath containing in aqueous solution about 1.5% of a fixing salt, about 1.5% of an alkaline salt of an organic oxy-acid, and about 105

110

- 0.5% of an ortho-phosphate of an alkali metal, the said fixing salt consisting in an alkaline salt of the most oxygenated oxide of a metal capable of forming at least one oxide soluble in an alkaline solution and a less oxygenated oxide insoluble in such a solution. 80
2. A process for protecting aluminium, magnesium, zinc and their alloys against corrosion, which consists in forming a protecting layer on 10 articles made of these metals or alloys by the action of a hot bath containing in aqueous solution about 1.5% of both a phospho-chromate of an alkali metal and a sulpho-molybdate of an alkali metal, about 0.5% of an ortho-phosphate of an 15 alkali metal and about 1.5% of an alkaline salt of an organic oxy-acid. 90
3. A process for protecting aluminium, magnesium, zinc and their alloys against corrosion, which consists in forming a protection layer on 20 articles made of these metals or alloys by the action of a hot bath containing in aqueous solution about 1.5% of both a phospho-chromate of an alkali metal and a sulpho-molybdate of an alkali metal, about 0.5% of an ortho-phosphate of an 25 alkali metal, about 1.5% of a carbonate of an alkali metal and about 1.5% of an alkaline salt of an organic oxy-acid. 100
4. A product adapted to be dissolved in water for the treatment of articles made of aluminium, magnesium, zinc and the like in order to protect 30 them against corrosion, this product being constituted by a mixture comprising about 1.5% of both a phospho-chromate of an alkali metal and a sulpho-molybdate of an alkali metal, about 0.5% of an ortho-phosphate of an alkali metal, about 1.5% of a carbonate of an alkali metal and about 1.5% of an alkaline salt of an organic oxy-acid. 105

PIERRE PRIER. 105

|    |     |
|----|-----|
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |